# EUROPEAN PATENT SPECIFICATION

(11) **EP 0 903 628 B1**
(45) Date of publication and mention of the grant of the patent: **07.07.2004**
(21) Application number: 98202655.1
(22) Date of filing: 06.08.1998
(51) Int. Cl.: G03C 1/498

(54) **Thermographic recording material with improved stability**
Thermographisches Aufzeichnungsmaterial mit erhöhter Stabilität
Matériau d'enregistrement thermographique à stabilité augmentée

(30) Priority: 06.12.1997 EP 97203834; 17.09.1997 EP 97202873; 17.09.1997 EP 97202872; 17.09.1997 EP 97202876; 17.09.1997 EP 97202877; 17.09.1997 EP 97202871; 17.09.1997 EP 97202875; 06.12.1997 EP 97203833; 06.06.1998 EP 98201963
(43) Date of publication of application: 24.03.1999
(73) Proprietor: AGFA-GEVAERT, 2640 Mortsel (BE)
(72) Inventor: Uyttendaele, Carlo, 2640 Mortsel (BE); Gilleir, Jan, 2640 Mortsel (BE); Geuens, Ingrid, 2640 Mortsel (BE); Hoogmartens, Ivan, 2640 Mortsel (BE)

(56) References cited:
- EP-A- 0 754 969
- EP-A- 0 810 467
- EP-A- 0 848 286
- EP-A- 0 851 285
- US-A- 2 910 377

## Description

### Field of the invention

The present invention relates to a substantially light-insensitive thermographic recording material with improved stability.

### Background of the invention.

Thermography is concerned with materials which are substantially light-insensitive, but are sensitive to heat or thermographic. Most of the "direct" thermographic recording materials are of the chemical type. On heating to a certain conversion temperature, an irreversible chemical reaction takes place and a coloured image is produced. A wide variety of chemical systems has been suggested some examples of which have been given on page 138 of the book "Imaging Systems" by Kurt I. Jacobson-Ralph E. Jacobson, The Focal Press - London and New York (1976), describing the production of a silver metal image by means of a thermally induced oxidation-reduction reaction of a silver soap with a reducing agent.

In US 2,910,977 the following statement is made in the description in column 7, lines 23-27: "Stability towards exposure to light is improved by selecting highly purified materials; freedom from halides and sulfides is particularly important in the case of compositions involving silver salts." The disclosure in US 2,910,977 concerned thermographic recording materials coated from solvent media.

WO 94/16361 discloses a multilayer heat-sensitive material which comprises: a colour-forming layer comprising: a colour-forming amount of finely divided, solid colourless noble metal or iron salt of an organic acid distributed in a carrier composition; a colour developing amount of a cyclic or aromatic organic reducing agent, which at thermal copy and printing temperatures is capable of a colour-forming reaction with the noble metal or iron salt; and an image-toning agent; characterized in that (a) the carrier composition comprises a substantially water-soluble polymeric carrier and a dispersing agent for the noble metal or iron salt and (b) the material comprises a protective overcoating layer for the colour-forming layer.

Coating of thermographic recording materials from aqueous media is preferred over coating from solvent for ecological and economic reasons. However, the inventors of the present invention found that the choice of surfactants used in the production of thermographic recording materials using aqueous dispersions and solutions had a substantial effect upon the stability of the thermographic recording materials produced and on prints produced therewith.

### Objects of the invention.

It is therefore an object of the present invention to provide thermographic recording materials coated from aqueous media, which exhibit improved stability.

It is therefore another object of the present invention to provide thermographic recording materials, which are capable of producing thermographic prints which exhibit improved stability.

Further objects and advantages of the invention will become apparent from the description hereinafter.

### Summary of the invention

In view of the statement made in US 2,910,977 to the effect that freedom from halides is particularly important it is surprising that the halide concentration in the totality of surfactants present in thermographic recording materials coated from aqueous media can be as high as 500ppm without adversely affected the light-stability of thermographic recording materials coated from aqueous media.

A process is provided for producing a substantially light-insensitive thermographic recording material substantially exclusive of cationic surfactants in which at least one non-cationic surfactant is present, wherein said thermographic recording material comprises a support and a thermosensitive element containing a substantially light-insensitive silver salt of an aliphatic carboxylic acid known as a fatty acid, a reducing agent therefor in thermal working relationship therewith and a binder, comprising the steps of: producing an aqueous dispersion of said substantially light-insensitive silver salt of an aliphatic carboxylic acid known as a fatty acid; producing one or more aqueous coating compositions containing together said aqueous dispersion of the substantially light-insensitive silver salt of an aliphatic carboxylic acid known as a fatty acid, said reducing agent and said binder; and applying said one or more aqueous coating compositions to said support thereby forming after drying said thermosensitive element, characterized in that one or more of said aqueous dispersion of said substantially light-insensitive silver salt of an aliphatic carboxylic acid known as a fatty acid and said one or more aqueous coating compositions contain a non-cationic surfactant and all said non-cationic surfactants present in the thermographic recording material together have a non-fluoro-halide ion concentration of 1500 to 200ppm.

A substantially light-insensitive thermographic recording material obtained by the above-mentioned process is also provided.

Preferred embodiments of the present invention are disclosed in the detailed description of the invention.

### Detailed description of the invention.

In a preferred embodiment the substantially light-insensitive thermographic recording materials of the present invention are black and white thermographic recording materials.

### Aqueous

The term aqueous for the purposes of the present invention includes mixtures of water with water-miscible organic solvents such as alcohols e.g. methanol, ethanol, 2-propanol, butanol, iso-amyl alcohol etc.; glycols e.g. ethylene glycol; glycerine; N-methyl pyrrolidone; methoxypropanol; and ketones e.g. 2-propanone and 2-butanone etc.

### Substantially

By substantially light-insensitive is meant not intentionally light sensitive. By substantially solvent-free aqueous medium is meant that solvent, if present, is present in amounts below 10% by volume of the aqueous medium.

### Non-cationic surfactants

Surfactants are surface active agents which are soluble compounds which reduce the interfacial tension between a liquid and a solid. Cationic surfactants have not been found to be useful for this application due to their photographic activity and the use of halide counterions in most commercial surfactants.

Non-cationic surfactants aid the dispersion of ingredients which are insoluble in the particular dispersion medium. The thermographic recording materials of the present invention contain at least one non-cationic surfactant, which may be anionic, non-ionic or amphoteric.

In the present invention the expression: "all the non- cationic surfactants present in the thermographic recording material together have a particular non-fluoro-halide ion concentration in ppm's", means 10⁶ multiplied by the sum of the quantities of non-fluoro-halide ions in the different non-cationic surfactants present divided by the sum of the quantities of all the non-cationic surfactants present in the same units of weight as that used for the quantities of non-fluoro-halide ions.

In a preferred embodiment of the present invention all the non-cationic surfactants present in the thermographic recording material together have a non-fluoro-halide ion concentration of 1000ppm or less, with 500ppm or less being particularly preferred and 200ppm being especially preferred. It is also preferred that all the non-cationic surfactants present in the thermographic recording material together have a metal ion concentration of 500 ppm or less with 200 ppm or less being particularly preferred and specially preferably that all the non-cationic surfactants present in the thermographic recording material together have an alkali metal ion concentration of 200 ppm or less. The alkali metal ions are: sodium, potassium, lithium, rubidium and caesium.

The chloride ion and sodium ion concentrations determined by ionic chromatography for commercial non-cationic surfactants according to the present invention are given in table 1.

**Table 1:**

| Surfactant Nr | Type | SURFACTANT | [Cl⁻] [ppm] | [Na⁺] [ppm] |
|---|---|---|---|---|
| S01 | A | HOSTAPAL™ B | <50 | |
| S02 | A | MARLON™ A365 | <40 | 4300 |
| S03 | A | dodecyl sulfonic acid | <40 | <1000 |
| S04 | A | ULTRAVON™ W | 700 | 74468 |
| S05 | A | HOSTAPUR™ SAS 60 | <40 | |
| S06 | A | MARLON™ AS3 | <200 | <200 |
| S07 | N | ANTAROX™ CO 880 | <40 | |
| S08 | N | SURFYNOL™ CT111 | <40 | |
| S09 | N | ARKOPAL™ N 060 | <20 | |
| S10 | N | GAFAC™ RM 710 | <40 | <1000 |
| S11 | A | ALKANOL™ XC | 1600 | |
| S12 | A | sodium dodecyl sulfate | 6400 | |
| S13 | A | DOWFAX™ 2A1 | 2700 | |
| S14 | A | NIAPROOF™ ANIONIC 4 | 7800 | |
| S15 | A | HOSTA™ | 5970 | |
| S16 | A | MERSOLAT™ H76 | 17000 | |
| S17 | A | HOSTAPON™ T | 84000 | |
| S18 | N | AKYPO™ OP80) | 3442 | 1338 |
| S19 | N | AKYPO™ RLM 45 | 2700 | |
| A: anionic | | | | |
| N: non-ionic | | | | |
| Surfactant Nr. S01 = HOSTAPAL™ B, supplied as a 50% concentrate of a sodium trisalkylphenyl-polyethyleneglycol(EO 7-8)sulphate by HOECHST; | | | | |
| Surfactant Nr. S02 = MARLON™ A-365, supplied as a 65% concentrate of a sodium alkyl-phenylsulfonate by HÜLS; | | | | |
| Surfactant Nr. S03 = 4-dodecylbenzene sulfonic acid from ; | | | | |
| Surfactant Nr. S04 = ULTRAVON™ W, supplied as a 75-85% concentrate of a sodium arylsulfonate by CIBA-GEIGY; | | | | |
| Surfactant Nr. S05 = HOSTAPUR™SAS, supplied as a 60% concentrate of a secondary alkanesulfonate by HOECHST; | | | | |
| Surfactant Nr. S06 = MARLON™ AS3, supplied as a 98% concentrate of an alkylphenylsulfonic acid by HÜLS; | | | | |
| Surfactant Nr. S07 = ANTAROX™ CO 880,a nonyl-phenyl-oxy-polyethyleneglycol(EO 30), from GAF; | | | | |
| Surfactant Nr. S08 = SURFYNOL™ CT111, a nonionic surfactant supplied by AIR PRODUCTS; | | | | |
| Surfactant Nr. S09 = ARKOPAL™ N060 (previously HOSTAPAL™ W), a nonylphenylpolyethylene-glycol from HOECHST. | | | | |
| Surfactant Nr. S10 = GAFAC™ RM710, a complex organic phosphate ester from GAF. | | | | |
| Surfactant Nr. S11 = ALKANOL™ XC, supplied as a 90% concentrate of a sodium nonylnaphthalene-sulfonate by DU PONT; | | | | |
| Surfactant Nr. S12 = sodium dodecyl sulphate from | | | | |
| Surfactant Nr. S13 = DOWFAX™ 2A1, supplied as a 45% concentrate of a disodium salt of di(decyl-sulfo-phenyl)ether by DOW CORNING; | | | | |
| Surfactant Nr. S14 = NIAPROOF ANIONIC™ 4, supplied as a 27% concentrate of a sodium 1-(2'-ethylbutyl)-4-ethylhexylsulphate by NIACET; | | | | |
| Surfactant Nr. S15 = HOSTA, supplied as a 95% concentrate of purified sodium salt of N-methyl-N-2-sulfoethyloleylamide, from HOECHST; | | | | |
| Surfactant Nr. S16 = MERSOLAT™ H76 (previously MERSOLAT™ H80), supplied as a 76% concentrate of a sodium pentadecylsulfonate by BAYER; | | | | |
| Surfactant Nr. S17 = HOSTAPON™ T, supplied as a 40% concentrate of a sodium salt of N-methyl-N-2-sulfoethyloleylamide by HOECHST; | | | | |
| Surfactant Nr. S18 = AKYPO™ OP80, supplied as an 80% concentrate of an octyl-phenyl-oxy-polyethyleneglycol(EO 8)acetic acid by CHEMY; | | | | |
| Surfactant Nr. S19 = AKYPO™ RLM45, supplied as a 85% concentrate of a monoethanolamine salt of a polyethyleneglycol-substituted fatty acid, by CHEMY; | | | | |

It is obvious that according to the thermographic recording materials of the present invention, surfactants S11 to S19 can only be used in combination with much larger quantities of surfactants with much lower chloride ion concentration, so that the overall chloride ion concentration in the surfactants present does not exceed 500ppm.

### Thermosensitive element

According to the present invention, a substantially light-insensitive thermographic recording material is provided comprising a thermosensitive element including a substantially light-insensitive organic silver salt, an organic reducing agent therefor in thermal working relationship therewith and a binder. The element may comprise a layer system in which the ingredients are dispersed in different layers, with the proviso that the substantially light-insensitive organic silver salt and the organic reducing agent are in thermal working relationship with one another i.e. during the thermal development process the reducing agent must be present in such a way that it is able to diffuse to the substantially light-insensitive organic silver salt particles so that reduction of the organic silver salt can take place. The thickness of the thermosensitive element is preferably in the range of 1 to 50 µm.

### Organic silver salts

Preferred substantially light-insensitive silver salts of aliphatic carboxylic acids known as fatty acids have an aliphatic carbon chain with at least 12 C-atoms, e.g. silver laurate, silver palmitate, silver stearate, silver hydroxystearate, silver oleate and silver behenate, which silver salts are also called "silver soaps". Silver salts of modified aliphatic carboxylic acids with thioether group as described e.g. in GB-P 1,111,492 and other organic silver salts as described in GB-P 1,439,478, e.g. silver benzoate, may likewise be used to produce a thermally developable silver image. Combinations of different organic silver salts may also be used in the present invention.

### Preparation of aqueous dispersions of silver behenate-containing particles in the substantial absence of solvent

The aqueous dispersion of the substantially light-insensitive salt is preferably produced using a production process for a dispersion of particles of substantially light-insensitive organic silver salt including silver behenate in an aqueous medium comprising the steps of: i) producing an aqueous dispersion of one or more organic acids including behenic acid and a salt of an alkylarylsulfonate; ii) substantially neutralizing the organic acids with aqueous alkali thereby forming organic acid salts including a behenic acid salt; (iii) adding an aqueous solution of a silver salt to completely convert the organic acid salts into their silver salts including silver behenate, characterized in that the anionic surfactant is present in a molar ratio with respect to organic acid greater than 0.15 and the silver salt is added at a rate between 0.025mol/mol organic silver salt·min and 2.25mol/mol organic silver salt·min. In preferred embodiments of the production process for a dispersion of particles of substantially light-insensitive organic silver salt including silver behenate in an aqueous medium the anionic surfactant is present in a molar ratio with respect to organic carboxylic acid greater than 0.25 and the silver salt is added at a rate between 0.03mol/mol organic silver salt·min and 0.7mol/mol organic silver salt·min, with a molar ratio of anionic surfactant with respect to organic acid greater than 0.3 and a rate of silver salt addition of between 0.04mol/mol organic silver salt·min and 0.3mol/mol organic silver salt·min being particularly preferred.

In a preferred embodiment step (iii) of the production process of the present invention is carried out such that part the solution of acid salts produced in step (ii) of the process is present in the reaction vessel prior to silver salt solution addition and part thereof is added simultaneously with the addition of the silver salt solution, with about 25 to 50% of the solution of acid salts produced in step (ii) being in the reaction vessel prior to silver salt addition being particularly preferred.

The above-described production process for a dispersion of particles of substantially light-insensitive organic silver salt including silver behenate in an aqueous medium the pH used must be sufficiently low to avoid the oxidation of silver ions to silver oxide or silver hydroxide for which a pH below 10 is usually required, the process temperature is chosen such that it is above the melting point of the organic acid(s) used which in the case of behenic acid means a temperature of about 80 to 85°C, must be carried out with stirring, the stirring rate being dependent upon the size of the stirrer relative to the reaction vessel, the type of stirrer used, avoidance of silver oxide or silver hydroxide formation due to insufficient mixing and avoidance of foaming, and being usually between 200 and 1000rpm and a slight excess of an organic acid, for example behenic acid with e.g. 2 mol% excess being preferred.

The size of the silver acid salts particles containing silver behenate can be varied by varying the rate of silver salt addition, the concentration of anionic surfactant and the temperature, the equivalent diameter of the particles increasing with decreasing addition rate, decreasing anionic surfactant concentration and increasing temperature.

### Film-forming binders of the thermosensitive element

The layer containing the organic silver salt is applied from an aqueous medium containing a water-dispersible binder and/or a water dispersible binder.

Suitable water-soluble film-forming binders for use in thermosensitive element according to the present invention are: polyvinyl alcohol, polyacrylamide, polymethacrylamide, polyacrylic acid, polymethacrylic acid, polyvinylpyrrolidone, polyethyleneglycol, proteinaceous binders such as gelatin, modified gelatins such as phthaloyl gelatin, polysaccharides, such as starch, gum arabic and dextran and water-soluble cellulose derivatives. A preferred water-soluble binder for use in the thermographic and photothermographic recording materials of the present invention is gelatin.

Suitable water-dispersible binders for use in the thermographic and photothermographic recording materials of the present invention may be any water-insoluble polymer It should be noted that there is no clear cut transition between a polymer dispersion and a polymer solution in the case of very small polymer particles resulting in the smallest particles of the polymer being dissolved and those slightly larger being in dispersion. Preferred water-dispersible binders for use according to the present invention are water-dispersible film-forming polymers with covalently bonded ionic groups selected from the group consisting of sulfonate, sulfinate, carboxylate, phosphate, quaternary ammonium, tertiary sulfonium and quaternary phosphonium groups. Further preferred water-dispersible binders for use according the the present invention are water-dispersible film-forming polymers with covalently bonded moieties with one or more acid groups.

The weight ratio of binder used according to the present invention to organic silver salt weight is preferably in the range of 0.2 to 6.

### Thermal solvents

The above mentioned binders or mixtures thereof may be used in conjunction with waxes or "heat solvents" also called "thermal solvents" or "thermosolvents" improving the reaction speed of the redox-reaction at elevated temperature. By the term "heat solvent" in this invention is meant a non-hydrolyzable organic material which is in a solid state in the recording layer at temperatures below 50°C, but upon heating becomes a plasticizer for the recording layer and/or a liquid solvent for at least one of the redox-reactants.

### Organic reducing agents

Suitable organic reducing agents for the reduction of organic silver salt particles containing silver stearate are organic compounds containing at least one active hydrogen atom linked to O, N or C, such as is the case with, aromatic di- and tri-hydroxy compounds; aminophenols; METOL (tradename); p-phenylene-diamines; alkoxynaphthols, e.g. 4-methoxy-1-naphthol described in US-P 3,094,41; pyrazolidin-3-one type reducing agents, e.g. PHENIDONE (tradename); pyrazolin-5-ones; indan-1,3-dione derivatives; hydroxytetrone acids; hydroxytetronimides; hydroxylamine derivatives such as for example described in US-P 4,082,901; hydrazine derivatives; and reductones e.g. ascorbic acid; see also US-P 3,074,809, 3,080,254, 3,094,417 and 3,887,378.

Catechol-type reducing agents, i.e. reducing agents containing at least one benzene nucleus with two hydroxy groups (-OH) in ortho-position, such as catechol, 3-(3,4-dihydroxyphenyl) propionic acid, 1,2-dihydroxybenzoic acid, gallic acid and esters e.g. methyl gallate, ethyl gallate, propyl gallate, tannic acid, and 3,4-dihydroxy-benzoic acid esters are preferred, with those described in EP-B 692 733 and unpublished European Patent Application EP 97202872.4 being particularly preferred. Other suitable reducing agents are sterically hindered phenols, bisphenols and sulfonamidophenols.

Combinations of reducing agents may also be used that on heating become reactive partners in the reduction of the substantially light-insensitive organic silver salt containing silver stearate. For example, combinations of reducing agents with sulfonamidophenols are described in the periodical Research Disclosure, February 1979, item 17842, in US-P 4,360,581 and 4,782,004, and in EP-A 423 891 and combinations of sterically hindered phenols with sulfonyl hydrazide reducing agents such as disclosed in US-P 5,464,738; trityl hydrazides and formyl-phenyl-hydrazides such as disclosed in US-P 5,496,695; trityl hydrazides and formyl-phenyl-hydrazides with diverse auxiliary reducing agents such as disclosed in US-P 5,545,505, US-P 5.545.507 and US-P 5,558,983; acrylonitrile compounds as disclosed in US-P 5,545,515 and US-P 5,635,339; and 2-substituted malonodialdehyde compounds as disclosed in US-P 5,654,130. Organic reducing metal salts, e.g. stannous stearate, have also been used in such reducing agent combinations, as disclosed in US-P 3,460,946 and 3,547,648, as have sterically hindered phenols and bisphenols, as described in US-P 4,001,026 and US-P 3,547,648 respectively.

### Toning agents

In order to obtain a neutral black image tone in the higher densities and neutral grey in the lower densities, thermographic recording materials according to the present invention may contain one or more toning agents. The toning agents should be in thermal working relationship with the substantially light-insensitive organic silver salt and reducing agents during thermal processing. Any known toning agent from thermography or photothermography may be used. Suitable toning agents are the phthalimides and phthalazinones within the scope of the general formulae described in US-P 4,082,901 and the toning agents described in US-P 3,074,809, US-P 3,446,648 and US-P 3,844,797. Particularly useful toning agents are the heterocyclic toner compounds of the benzoxazine dione or naphthoxazine dione type described in GB-P 1,439,478, US-P 3,951,660 and US-P 5,599,647.

### Dispersants

Suitable dispersants are natural polymeric substances, synthetic polymeric substances and finely divided powders, for example finely divided non-metallic inorganic powders such as silica.

### Stabilizers and antifoggants

In order to obtain improved shelf-life and reduced fogging, stabilizers and antifoggants may be incorporated into the thermographic recording materials of the present invention.

### Polycarboxylic acids and anhydrides thereof

According to the recording material of the present invention the thermosensitive element may comprise in addition at least one polycarboxylic acid and/or anhydride thereof in a molar percentage of at least 15 with respect to all the organic silver salt(s) present and in thermal working relationship therewith. The polycarboxylic acid may be aliphatic (saturated as well as unsaturated aliphatic and also cycloaliphatic) or an aromatic polycarboxylic acid. These acids may be substituted e.g. with alkyl, hydroxyl, nitro or halogen. They may be used in anhydride form or partially esterified on the condition that at least two free carboxylic acids remain or are available in the heat recording step.

### Other ingredients

In addition to the ingredients the substantially light-insensitive thermographic recording material may contain other additives such as free fatty acids, silicone oil, ultraviolet light absorbing compounds, white light reflecting and/or ultraviolet radiation reflecting pigments, silica, and/or optical brightening agents.

### Support

The support for the substantially light-insensitive thermographic recording material according to the present invention may be transparent, translucent or opaque and is preferably a thin flexible carrier made e.g. from paper, polyethylene coated paper or transparent resin film, e.g. made of a cellulose ester, e.g. cellulose triacetate, polypropylene, polycarbonate or polyester, e.g. polyethylene terephthalate. The support may be in sheet, ribbon or web form. The support may be made of an opacified resin composition.

### Subbing layer between the support and the thermosensitive element

A subbing layer may also be provided between the support and the thermosensitive element. In a preferred embodiment the subbing layer contains a binder, less than 20% by weight of silica and covalently bonded acid groups in the binder, if present, are either substantially present as free acid or substantially present as acid salts. In a further preferred embodiment the subbing layer contains a non-cationic surfactant.

It is particularly preferred that the subbing layer used in the thermographic recording materials of the present invention contain less than 40ppm of free choride ions, with less than 10ppm of free chloride ions being especially preferably.

Preferred ingredients for the subbing layer used in the thermographic recording materials of the present invention are a polymer latex, polyethylene wax and hydrolyzed polyalkoxysilanes. By the term polyalkoxysilane is meant a silane with a least two hydrolyzable alkoxy-groups.

### Protective layer

A protective layer may also be provided for the thermosensitive element. In a preferred embodiment this protective layer contains a non-cationic surfactant. In general the protective layer protects the thermosensitive element from atmospheric humidity and from surface damage by scratching etc. and prevents direct contact of printheads or heat sources with the recording layers. Protective layers for thermosensitive elements which come into contact with and have to be transported past a heat source under pressure, have to exhibit resistance to local deformation and good slipping characteristics during transport past the heat source during heating.

The protective layer may comprise a dissolved lubricating material and/or particulate material, e.g. talc particles, optionally protruding therefrom. Examples of suitable lubricating materials are a surface active agent, a liquid lubricant, a solid lubricant or mixtures thereof, which may be used with or without a polymeric binder. Suitable slipping layer compositions are described, for example, in US 5,587,350, US 5,536,696, US 5,547,914, WO 95/12495, EP-A 775 592 and EP-A 775 595.

### Coating

The coating of any layer of the substantially light-insensitive thermographic recording materials of the present invention may proceed by any coating technique e.g. such as described in Modern Coating and Drying Technology, edited by Edward D. Cohen and Edgar B. Gutoff, (1992) VCH Publishers Inc., 220 East 23rd Street, Suite 909 New York, NY 10010, USA.

### Thermographic printing

Thermographic imaging is carried out by the image-wise application of heat either in analogue fashion by direct exposure through an image of by reflection from an image, or in digital fashion pixel by pixel either by using an infra-red heat source, for example with a Nd-YAG laser or other infra-red laser, or by direct thermal imaging with a thermal head.

In thermal printing, image signals are converted into electric pulses and then through a driver circuit selectively transferred to a thermal printhead. The thermal printhead consists of microscopic heat resistor elements, which convert the electrical energy via the Joule effect into heat, which is transferred to the surface of the thermographic recording material wherein the chemical reaction resulting in the development of a black and white image takes place. Such thermal printing heads may be used in contact or close proximity with the recording layer. The operating temperature of common thermal printheads is in the range of 300 to 400°C and the heating time per picture element (pixel) may be less than 1.0 ms, the pressure contact of the thermal printhead with the recording material being e.g. 200-500g/cm² to ensure a good transfer of heat.

In order to avoid direct contact of the thermal printing heads with a recording layer not provided with an outermost protective layer, the image-wise heating of the recording layer with the thermal printing heads may proceed through a contacting but removable resin sheet or web wherefrom during the heating no transfer of recording material can take place.

The image signals for modulating the laser beam or current in the micro-resistors of a thermal printhead are obtained directly e.g. from opto-electronic scanning devices or from an intermediary storage means, optionally linked to a digital image work station wherein the image information can be processed to satisfy particular needs.

Activation of the heating elements can be power-modulated or pulse-length modulated at constant power. EP-A 654 355 describes a method for making an image by image-wise heating by means of a thermal head having energizable heating elements, wherein the activation of the heating elements is executed duty cycled pulsewise.

When used in thermographic recording operating with thermal printheads the thermographic recording materials are not suitable for reproducing images with fairly large number of grey levels as is required for continuous tone reproduction. EP-A 622 217 discloses a method for making an image using a direct thermal imaging element producing improvements in continuous tone reproduction.

Image-wise heating of the thermographic recording material can also be carried out using an electrically resistive ribbon incorporated into the material. Image- or pattern-wise heating of the thermographic recording material may also proceed by means of pixelwise modulated ultra-sound, using e.g. an ultrasonic pixel printer as described e.g. in US-P 4,908,631.

### Industrial application

Substantially light-insensitive thermographic recording materials according to the present invention may be used for both the production of transparencies, for example in the medical diagnostic field in which black-imaged transparencies are widely used in inspection techniques operating with a light box, and reflection type prints, for example in the hard copy field. For such applications the support will be transparent or opaque, i.e. having a white light reflecting aspect. Should a transparent base be used, the base may be colourless or coloured, e.g. with a blue colour for medical diagnostic applications.

The following examples and comparative examples illustrate the present invention. The percentages and ratios used in the examples and compositions of the ingredients are by weight unless otherwise indicated.

### i) subbing layer ingredients:

- PAREZ RESIN™ 707:: a 80% solids melamine-formaldehyde resin from AMERICAN CYANAMID;
- HORDAMER™ PE02:: a 40% aqueous dispersion of polyethylene from HOECHST;
- R10985:: a calcium-containing medium viscosity gelatin from ROUSSELOT;
- KIESELSOL 100F:: a 36% aqueous dispersion of colloidal silica from BAYER;
- KIESELSOL 300F:: a 30% aqueous dispersion of colloidal silica from BAYER;
- PMMA:: a 20% aqueous dispersion of polymethylmethacrylate particles 2µm in diameter

### ii) thermosensitive element ingredients:

- K7598 =: type 7598, a calcium-free gelatin from AGFA-GEVAERT GELATINEFABRIEK vorm. KOEPFF & SÖHNE;
- K17881 =: type 17881, a calcium-free gelatin with low potassium ion, sodium ion and chloride-ion concentrations from AGFA-GEVAERT GELATINEFABRIEK vorm. KOEPFF & SÖHNE;
- AgB =: silver behenate
- B79 =: BUTVAR™ B79, a polyvinyl butyral from MONSANTO
- R01 =: ethyl 3,4-dihydroxybenzoate, a reducing agent
- T01 =: 7-(ethylcarbonato)benzo[e][1,3]oxazine-2,4-dione, a toning agent
- T02 =: benzo[e][1,3]oxazine-2,4-dione, a toning agent
- Surfactant Nr. S19 =: ammonium dodecylphenylsulfonate with a Cl⁻ ion concentration below the detection limit of 20ppm;
- Surfactant Nr. S20 =: ammonium dodecylphenylsulfonate with 50ppm Cl⁻;
- Surfactant Nr. S21 =: ammonium dodecylphenylsulfonate with 200ppm Cl⁻;
- Surfactant Nr. S22 =: ammonium dodecylphenylsulfonate with 500ppm Cl⁻;
and the following latexes:

| polymer Latex nr | B [%] | IP [%] | BA [%] | S [%] | MMA [%] | IA [%] | MAA [%] | AA [%] |
|---|---|---|---|---|---|---|---|---|
| 1# | 47.5 | - | - | - | 47.5 | 5 | - | - |
| 2 | 49 | - | - | - | 49 | 2 | - | - |
| 3 | - | 47.5 | - | - | 47.5 | 5 | - | - |
| 4 | - | - | 43 | 55 | - | 2 | - | - |
| 5 | - | - | 43 | 55 | - | - | 2 | - |
| 6 | - | - | 47 | 46 | - | - | 7 | - |
| 7 | - | - | 44 | 54 | - | - | 2 | - |
| 8 | - | - | 47.5 | 47.5 | - | - | - | 5 |
| 9* | 50 | - | - | - | 50 | - | - | - |

| | | | | | | | | |
|---|---|---|---|---|---|---|---|---|
| # contains 1% of Surfactant Nr S01 versus monomers polymerized | | | | | | | | |
| * contains of 2% of Surf. Nr S04 & 0.8% of Surf. Nr S17 vs monomers polymerized where: B = butadiene; IP = isoprene; BA = butyl acrylate; EA = ethyl acrylate; S = styrene; MMA = methyl methacylate; IA = itaconic acid; MAA = methacrylic acid; and AA = acrylic acid. | | | | | | | | |

### REFERENCE EXAMPLES 1 to 10 and COMPARATIVE EXAMPLES 1 & 2

### Preparation of subbing layer

A 0.34mm thick polyethylene terephthalate sheet was coated to a thickness of 0.1mm with a composition which after drying and longitudinal and transverse stretching produced a 175 µm thick support coated on with the following subbing-layer composition expressed as the coating weights of the ingredients present:

| | |
|---|---|
| # copolymer of terephthalic acid/isophthalic acid/sulfoisophthalic acid/ethylene glycol (26.5/20/3.5/50)* | 37.0mg/m² |
| # copolymer latex of ethyl acrylate/methacrylic acid (80/20) | 3.0mg/m² |
| # HORDAMER™ PE02 | 1.0mg/m² |
| # PAREZ RESIN™ 707 | 7.0mg/m² |

| | |
|---|---|
| * contains 7.1% of Surf. Nr S18 & 1.98% of Surf. Nr S01 vs monomers polymerized | |

### Preparation of a silver behenate dispersion

9000g of silver behenate were added with stirring to 9000g of a 10% aqueous solution of Surfactant Nr S02 diluted with 20,146g of deionized water and the mixture stirred for 30 minutes with a KOTTHOFF™ stirrer. The resulting dispersion was then passed four times through a Type M110F high pressure homogenizer from MICROFLUIDICS™ Corporation at a pressure of 400 bar to obtain a finely divided aqueous silver behenate dispersion.

### Preparation of a tone modifier dispersion

The tone modifier dispersion was prepared by first dissolving 8.8g of K7598 in 71.4g of deionized water by first adding the gelatin, then allowing the gelatin to swell for 30 minutes and finally heating to 50°C. 20 g of T01 was added with ULTRA-TURRAX™ stirring to this gelatin solution at 50°C, and the stirring continued for a further 5 minutes. Finally the resulting dispersion was pumped through a DYNOMILL™ for 2 hours to produce the final tone modifier dispersion containing: 20% of T01 and 8.8% of K7598.

### Preparation of the silver behenate emulsion layers

The coating dispersions for the thermographic recording materials of REFERENCE EXAMPLES 1 to 10 and COMPARATIVE EXAMPLES 1 & 2 were prepared by first dissolving 1.927g of K7598 in deionized water at 38°C (for the quantity of water see table 1), then adding with stirring to the warm K7598 solution: first 19.0g of the silver behenate dispersion, then 5.68g of the tone modifier dispersion as flakes followed by 15 minutes stirring, then the latex dispersion (for quantity, concentration and type see table 1), then 11.23g of an aqueous ethanol solution containing 0.92g of R01 and 0.62g of boric acid and finally 1.310g of a 3.7% by weight solution of formaldehyde to produce 60g of a dispersion containing: 7.47% of silver behenate, 0.75% of Surfactant Nr S02, 4.04% of K7598, 2.98% of polymer latex, 1.53% of R01, 1.03% of boric acid, 1.92% of T01 and 0.08% of formaldehyde.

**Table 1**

| Comparative Example number | Quantity of water [g] | polymer latex | | |
|---|---|---|---|---|
| | | number | concentration [%] | weight [g] |
| 1 | 11.653 | S11 | 19.4 | 9.200 |
| 2 | 11.653 | S11 | 19.4 | 9.200 |

| Reference Example number | | | | |
|---|---|---|---|---|
| 1 | 14.713 | 1 | 29.1 | 6.140 |
| 2 | 14.903 | 1* | 30.0 | 5.950 |
| 3 | 14.903 | 1# | 30.0 | 5.950 |
| 4 | 14.713 | 1# | 29.1 | 6.140 |
| 5 | 10.723 | 4 | 17.6 | 10.130 |
| 6 | 10.973 | 4^{a} | 18.1 | 9.880 |
| 7 | 11.083 | 5 | 18.3 | 9.770 |
| 8 | 16.643 | 6 | 42.4 | 4.210 |
| 9 | 16.823 | 7 | 44.2 | 4.040 |
| 10 | 10.683 | 8 | 17.5 | 10.170 |

| | | | | |
|---|---|---|---|---|
| * pH adjusted to 5.5 | | | | |
| # pH adjusted to 5 | | | | |
| a = no buffer | | | | |

The resulting emulsions were then doctor blade-coated to a wet thickness of 60µm at a blade setting of 100µm onto the 175µm thick subbed polyethylene terephthalate support and dried for 10 minutes at 50°C, producing a silver behenate coverage of about 4.0g/m².

### Thermographic printing

The printer was equipped with a thin film thermal head with a resolution of 300 dpi and was operated with a line time of 19ms (the line time being the time needed for printing one line). During this line time the printhead received constant power. The average printing power, being the total amount of electrical input energy during one line time divided by the line time and by the surface area of the heat-generating resistors was 1.6 mJ/dot being sufficient to obtain maximum optical density in each of the substantially light-insensitive thermographic recording materials of REFERENCE EXAMPLES 1 to 10 and COMPARATIVE EXAMPLES 1 & 2.

The maximum densities, Dₘₐₓ, and minimum densities, Dₘᵢₙ, of the prints given in table 2 were measured through visible or blue filters with a MACBETH™ TR924 densitometer in the grey scale step corresponding to data levels of 64 and 0 respectively and are given in table 2.

### Archivability test

The achivability of prints made with the substantially light-insensitive thermographic recording materials of REFERENCE EXAMPLES 1 to 10 and COMPARATIVE EXAMPLES 1 & 2 was evaluated on the basis of the observed changes in minimum density, Dₘᵢₙ, upon heating the prints at 35°C in a relative humidity (RH) of 80% for 3 days in the dark. The results of these tests are also given in table 2.

### Light box test

The stability of the image background of the prints made with the substantially light-insensitive thermographic recording materials of REFERENCE EXAMPLES 1 to 10 and COMPARATIVE EXAMPLES 1 & 2 was evaluated on the basis of the change in minimum (background) density measured through a blue filter using a MACBETH™ TR924 densitometer upon exposure on top of the white PVC window of a specially constructed light-box placed for 3 days in a VÖTSCH conditioning cupboard set at 30°C and a relative humidity (RH) of 85%. Only a central area of the window 550mm long by 500mm wide was used for mounting the test materials to ensure uniform exposure.

The stainless steel light-box used was 650mm long, 600mm wide and 120mm high with an opening 610mm long and 560mm wide with a rim 10mm wide and 5mm deep round the opening, thereby forming a platform for a 5mm thick plate of white PVC 630mm long and 580mm wide, making the white PVC-plate flush with the top of the light-box and preventing light loss from the light-box other than through the white PVC-plate. This light-box was fitted with 9 Planilux™ TLD 36W/54 fluorescent lamps 27mm in diameter mounted length-wise equidistantly from the two sides, with the lamps positioned equidistantly to one another and the sides over the whole width of the light-box and with the tops of the fluorescent tubes 30mm below the bottom of the white PVC plate and 35mm below the materials being tested. The results are summarized in table 2.

**Table 2:**

| Comparative example number | AgB coverage [g/m²] | Surfactant(s) | | FRESH PRINT | | Archiv-ability ΔDₘᵢₙ vis/blue after 3d at 35°C/80%RH | Light box: **Δ**Dₘᵢₙ vis/blue after 3d at 30°C/85%RH |
|---|---|---|---|---|---|---|---|
| | | Nr (s) | [Cl⁻] ppm | Dₘₐₓ vis/blue | Dₘᵢₙ vis/blue | | |
| 1 | 3.98 | S01, S02, S04, S17,S18 | 2499 | 4.61/4.54 | 0.08/0.11 | 0.07/0.13 | 0.09/0.35 |
| 2 | 4.08 | S01, S02, S04, S17,S18 | 2499 | 4.62/4.48 | 0.06/0.08 | 0.02/0.03 | 0.13/0.20 |

| Reference number | | | | | | | |
|---|---|---|---|---|---|---|---|
| 1 | 3.40 | S01,S02,S18 | 26-66 | 3.47/3.43 | 0.09/0.11 | 0.01/0.02 | 0.03/0.09 |
| 2 | 3.87 | S01.S02.S18 | 23-63 | 4.54/4.36 | 0.08/0.11 | 0.02/0.03 | 0.03/0.08 |
| 3 | 4.24 | S01.S02.S18 | 21-61 | 2.72/2.79 | 0.10/0.13 | 0.00/0.01 | 0.04/0.08 |
| 4 | 4.24 | S01.S02.S18 | 21-61 | 3.65/3.63 | 0.08/0.10 | 0.00/0.01 | 0.04/0.08 |
| 5 | 4.21 | S01.S02,S18 | 21-61 | 4.14/3.75 | 0.09/0.11 | 0.00/0.01 | 0.03/0.06 |
| 6 | 4.69 | S01, S02, S18 | 19-59 | 4.03/3.98 | 0.07/0.09 | 0.00/0.01 | 0.04/0.08 |
| 7 | 4.45 | S01, S02, S18 | 20-60 | 3.01/3.23 | 0.09/0.11 | 0.00/0.01 | 0.03/0.07 |
| 8 | 4.53 | S01.S02.S18 | 20-60 | 4.08/4.14 | 0-06/0.08 | 0.02/0.02 | 0.04/0.07 |
| 9 | 4.40 | S01, S02, S18 | 20-60 | 4.53/4.43 | 0.07/0.10 | 0.02/0.03 | 0.05/0.09 |
| 10 | 5.03 | S01.S02.S18 | 18-58 | 3.14/3.18 | 0.08/0.10 | 0.00/0.01 | 0.03/0.06 |

The results of the archivability and light box tests show that the stability in light box tests of prints made with the substantially light-insensitive thermographic recording materials of REFERENCE EXAMPLES 1 to 10 in which Surfactant Nr S02 is used with a chloride ion concentration of less than 40 ppm are superior to those of the substantially light-insensitive thermographic recording material of COMPARATIVE EXAMPLES 1 & 2 in which Surfactant Nr S02 with a chloride ion concentration of less than 40 ppm is present together with the Surfactant Nr S17 with a chloride ion concentration of 84000 ppm from the Latex Nr 09 used in their preparation. These results show that the integral chloride ion concentration of the non-cationic surfactants used is important in determining the stability of the prints prepared with substantially light-insensitive thermographic recording materials.

### REFERENCE EXAMPLES 19 to 22 & COMPARATIVE EXAMPLES 6 & 7

### Preparation of silver behenate dispersions in an aqueous medium in the absence of organic solvent using a single jet process

Aqueous dispersions of the silver behenate types VI to IX of REFERENCE EXAMPLES 19 to 22 and of silver behenate types X & XI of COMPARATIVE EXAMPLES 6 & 7 respectively were produced as described for silver behenate types I to V of REFERENCE EXAMPLES 12 to 16 except as mentioned in table 7 below. The volume average particle size as determined by a Coulter LS230 diffractometer is also given in table 7.

**Table 7:**

| Reference example number | AgB type | Surfactant | | Temperature [°C] | mol AgNO₃/ mol AgB·min | ultrafiltration | | average particle size [µm] |
|---|---|---|---|---|---|---|---|---|
| | | Nr | g./g Hbeh | | | residual conductivity [mS/cm] | % AgB dispersion | |
| 19 | VI | S02 | 0.395 | 80 | 6.25×10⁻³ | 2.20 | 22.46 | 0.459 |
| 20 | VII | S05 | 0.362 | 80 | 6.25×10⁻³ | 1.9 | 18.4 | 0.463 |
| 21 | VIII | S05 | 0.362 | 80 | 6.25×10⁻³ | 1.4 | 17.5 | 0.260 |
| 22 | IX | S01 | 0.403 | 80 | 6.25×10⁻³ | 1.9 | 23.1 | 0.615 |

| Comparative example number | | | | | | | | |
|---|---|---|---|---|---|---|---|---|
| 6 | X | S18 | 0.715 | 80 | 6.25×10⁻³ | 1.8 | 16.4 | 0.438 |
| 7 | XI | S12 | 0.440 | 80 | 6.25×10⁻³ | 2.6 | 19.4 | - |

These dispersions of silver behenate were directly used in the preparation of thermographic recording materials comprising thermographic elements coated from aqueous media.

### Preparation of coating dispersion

3.45g of K17881 was allowed to swell for 30 minutes in 4.8g of a 5% aqueous solution of adipic acid adjusted to pH 5.3 with ammonia diluted with water (see table 8 for quantity) and the swollen gelatin heated up to 36°C. The following ingredients were then added with stirring: 4.875 of the tone modifier dispersion used in REFERENCE EXAMPLES 1 to 10 and COMPARATIVE EXAMPLES 1 & 2 were added, followed by 5 minutes stirring before the silver behenate dispersion, at a temperature of 36°C, was added first about 2g then stirring for 5 minutes before adding the rest (for quantity, silver behenate concentration & nature of the dispersion agent see table 8), followed by 10 minutes stirring before 11.150g of an aqueous solution containing 2.78% of boric acid, 8.17% of R01 and 15.23% of ethanol was added was added and finally 1g of an aqueous solution containing 19.2% of formaldehyde and 6.75% of methanol was added followed by 5 minutes stirring.

**Table 8:**

| Reference example number | AgB type | quantity of deionized water [g] | AgB dispersion | | | |
|---|---|---|---|---|---|---|
| | | | Surfactant Nr | g Surfactant/ g AgB | AgB conc [wt. %] | quantity of AgB dispersion [g] |
| 19 | VI | 12.825 | S02 | 0.128 | 22.46 | 21.90 |
| 20 | VII | 7.875 | S05 | 0.21 | 18.4 | 26.85 |
| 21 | VIII | 6.525 | S05 | 0.17 | 17.5 | 28.20 |
| 22 | IX | 13.325 | S01 | 0.22 | 23.1 | 21.40 |

| Comparative example number | | | | | | |
|---|---|---|---|---|---|---|
| 6 | X | 4.525 | S18 | 0.31 | 16.4 | 30.20 |
| 7 | XI | 9.325 | S12 | 0.22 | 19.4 | 25.40 |

The resulting silver behenate emulsions were then doctor blade-coated onto a 175µm thick polyethylene terephthalate support subbed with the subbing layer described for REFERENCE EXAMPLES 1 to 10 and COMPARATIVE EXAMPLES 1 & 2 to produce the coating weights of silver given in table 9.

### Thermographic evaluation

The thermographic recording materials of REFERENCE EXAMPLES 19 to 22 and COMPARATIVE EXAMPLES 6 & 7 were printed and the prints evaluated as described for REFERENCE EXAMPLES 1 to 10 and COMPARATIVE EXAMPLES 1 & 2. The maximum and minimum densities of the prints obtained with the thermographic recording materials of REFERENCE EXAMPLES 19 to 22 and COMPARATIVE EXAMPLES 6 & 7 measured through a blue filter with a MACBETH™ TR924 densitometer for grey scale steps corresponding to data levels of 255 and 0 respectively are also given in table 9. The archivability tests and light box tests were carried out on the thermographic recording materials of REFERENCE EXAMPLES 19 to 22 and COMPARATIVE EXAMPLES 6 & 7 as described for REFERENCE EXAMPLES 1 to 10 and COMPARATIVE EXAMPLES 1 & 2. The results are summarized in table 9.

**Table 9:**

| Reference example number | AgBcoverage [g/m²] | Surfactant | | fresh | | Archivability (ΔDₘₐₓ/ΔDₘᵢₙ blue) after 3d/35°C/80% RH | Light box ΔDₘₐₓ/ΔDₘᵢₙ (blue) after 3d/30°C/85%RH |
|---|---|---|---|---|---|---|---|
| | | Nr | [Cl⁻] ppm | Dₘₐₓ blue | Dₘᵢₙ blue | | |
| 19 | 4.43 | S01.S02,S18 | 16-56 | 2.74 | 0.08 | +0.78/+0.02 | +0.23/+0.02 |
| 20 | 3.90 | S01.S05.S18 | 11-51 | 3.89 | 0.08 | +0.42/+0.02 | +0.27/+0.02 |
| 21 | 4.19 | S01,S05,S18 | 13-52 | 3.95 | 0.08 | +0.35/+0.01 | +0.07/+0.01 |
| 22 | 3.64 | S01,S18 | 11-61 | 4.08 | 0.08 | +0.29/+0.01 | -0.01/+0.01 |

| Comparative example number | | | | | | | |
|---|---|---|---|---|---|---|---|
| 6 | 4.40 | S01,S18 | 3440 | 4.24 | 0.09 | +0.14/+0.01 | +0.12/+0.41 |
| 7 | 4.95 | S01,S12,S18 | 6389 | 4.21 | 0.10 | +0.20/+0.07 | +0.12/+0.03 |

The results of the thermographic evaluation of the thermographic recording material of REFERENCE EXAMPLES 19 to 22 show lower increases in Dₘᵢₙ in archivability and light box tests, indicating higher stability, than those for the thermographic recording materials of COMPARATIVE EXAMPLES 6 & 7 which contain Surfactants with high chloride-ion concentrations (S18 and S12 respectively) in addition to Surfactant Nrs S01 and S08.

### REFERENCE EXAMPLES 23 to 26 & COMPARATIVE EXAMPLES 8 to 13

### Preparation of silver behenate dispersions

Silver behenate was added with stirring to an aqueous solution of different surfactants (for surfactant used see table 10) and the mixtures stirred for 30 minutes with a KOTTHOFF™ stirrer. The resulting dispersions were then ball milled to obtain a finely divided aqueous silver behenate dispersion with the quantities of surfactant with respect to silver behenate given in table 10.

**Table 10:**

| Reference example number | Surfactant | | AgB-concentration in dispersion [% by weight] |
|---|---|---|---|
| | Nr | g/g AgB | |
| 23 | S02 | 0.1 | 20.7 |
| 24 | S01 | 0.1 | 20.15 |
| 25 | S05 | 0.1 | 19.44 |
| 26 | S03 | 0.1 | 19.81 |

| Comparative example number | | | |
|---|---|---|---|
| 8 | S16 | 0.1 | 20.16 |
| 9 | S11 | 0.1 | 19.8 |
| 10 | S18 | 0.1 | 19.71 |
| 11 | S17 | 0.1 | 20.64 |
| 12 | S12 | 0.1 | 20.81 |
| 13 | S15 | 0.1 | 20.16 |

### Preparation of coating dispersion

3.67g of K17881 was allowed to swell in water (see table 11 for quantity) for 30 minutes and the swollen gelatin was heated up to 36°C. The following ingredients were then added with stirring: 4.434g of an aqueous dispersion of 6.63% of K7598 and 13.37% of phthalazinone, the resulting solution was then stirred for an additional 5 minutes before the silver behenate dispersion, at a temperature of 36°C, was added first about 2g then stirring for 5 minutes before adding the rest (for quantity, silver behenate concentration & nature of the dispersion agent see table 11), then 11.150g of an aqueous solution containing 2.78% of boric acid, 8.17% of R01 and 15.23% of ethanol was added and finally 1g of an aqueous solution containing 19.2% of formaldehyde and 6.75% of methanol was added followed by 5 minutes stirring.

**Table 11:**

| Reference example number | quantity of deionized water [g] | AgB dispersion | | |
|---|---|---|---|---|
| | | Surfactant Nr | concentration [% by wt.] | quantity [g] |
| 23 | 15.996 | S02 | 20.7 | 23.750 |
| 24 | 15.346 | S01 | 20.15 | 24.40 |
| 25 | 14.446 | S05 | 19.44 | 25.30 |
| 26 | 14.931 | S03 | 19.81 | 24.815 |

| Comparative example number | | | | |
|---|---|---|---|---|
| 8 | 15.346 | S16 | 20.16 | 24.40 |
| 9 | 14.946 | S11 | 19.8 | 24.80 |
| 10 | 14.746 | S18 | 19.71 | 25.00 |
| 11 | 15.896 | S17 | 20.64 | 23.85 |
| 12 | 36.121 | S12 | 20.81 | 23.625 |
| 13 | 15.371 | S15 | 20.16 | 24.375 |

The resulting silver behenate emulsions were then doctor blade-coated onto a 175µm thick subbed polyethylene terephthalate support to produce the coating weights of silver given in table 12.

### Thermographic evaluation

The thermographic recording materials of REFERENCE EXAMPLES 23 to 26 and COMPARATIVE EXAMPLES 8 to 13 were printed and the prints evaluated as described for REFERENCE 1 to 10 and COMPARATIVE EXAMPLES 1 & 2. The maximum and minimum densities of the prints obtained with the thermographic recording materials of REFERENCE EXAMPLES 23 to 26 and COMPARATIVE EXAMPLES 8 to 13 measured through a blue filter with a MACBETH™ TR924 densitometer for grey scale steps corresponding to data levels of 255 and 0 respectively are also given in table 12. The archivability tests and light box tests were carried out on the thermographic recording materials of REFERENCE EXAMPLES 23 to 26 and COMPARATIVE EXAMPLES 8 to 13 as described for REFERENCE EXAMPLES 1 to 10 and COMPARATIVE EXAMPLES 1 & 2. The results are summarized in table 12.

**Table 12**

| Reference example number | AgB coverage [g/m²] | Surfactant | | fresh | | Archivability (ΔDₘₐₓ/ΔDₘᵢₙ blue) after 3d at 35°C/80%RH | Light box: ΔDₘₐₓ/ΔDₘᵢₙ blue after 3d at 30°C/85%RH |
|---|---|---|---|---|---|---|---|
| | | Nr | [Cl⁻] ppm | Dₘₐₓ blue | Dₘᵢₙ blue | | |
| 23 | 3.87 | S01,S02,S18 | 23-63 | 4.12 | 0.07 | -0.01/-0.01 | -0.09/+0.02 |
| 24 | 3.82 | S01,S18 | 23-73 | 4.35 | 0.05 | -0.02/+0.00 | 0.00/+0.03 |
| 25 | 6.19 | S01,S05,S18 | 18-54 | 4.21 | 0.06 | +0.03/+0.00 | +0.01/+0.02 |
| 26 | 5.11 | S01,S03, S18 | 18-57 | 4.22 | 0.06 | -0.05/-0.01 | -0.12/+0.03 |

| Comparative example number | | | | | | | |
|---|---|---|---|---|---|---|---|
| 8 | 5.66 | S01, S16, S18 | 16916 | 4.05 | 0.11 | -0.14/-0.02 | -0.31/+0.11 |
| 9 | 4.11 | S01,S11,S18 | 1609 | 4.03 | 0.08 | -0.03/+0.00 | -0.22/+0.05 |
| 10 | 4.85 | S01,S18 | 3437 | 4.07 | 0.06 | +0.09/+0.02 | -0.11/+0.08 |
| 11 | 3.90 | S01,S17,S18 | 83333 | 4.13 | 0.09 | -0.30/+0.02 | -0.18/+0.15 |
| 12 | 4.06 | S01,S12, S18 | 6368 | 3.62 | 0.08 | -0.25/+0.01 | -0.44/+0.04 |
| 13 | 3.82 | S01,S15,S18 | 3600 | 4.25 | 0.06 | +0.07/+0.04 | -0.01/+0.06 |

The results of the thermographic evaluation of the thermographic recording material of REFERENCE EXAMPLES 23 to 26 show lower increases in Dₘᵢₙ in archivability and light box tests, indicating higher stability, than those for the thermographic recording materials of COMPARATIVE EXAMPLES 8 to 13 which contain Surfactants with high chloride-ion concentrations (S16, S11, S18, S17, S12 and S15 respectively)in addition to Surfactant Nrs S01 and S09 from the subbing layer of the support.

### REFERENCE EXAMPLES 27 and 28 and INVENTION EXAMPLES 1 and 2

### Preparation of silver behenate dispersions

Silver behenate was added with stirring to an aqueous solution of different surfactants (for surfactant used see table 16) and the mixtures stirred for 30 minutes with a KOTTHOFF™ stirrer. The resulting dispersions were then ball-milled to obtain a finely divided aqueous silver behenate dispersion with the quantities of surfactant with respect to silver behenate given in table 16.

**Table 16:**

| Reference example number | Surfactant | | | AgB-concentration in dispersion [% by weight] |
|---|---|---|---|---|
| | Nr | Cl⁻ concentration [ppm] | g 10% sol /g AgB | |
| 30 | S19 | <20 | 1 | 18.55 |
| 31 | S20 | 50 | 1 | 18.55 |

| Invention example number | | | | |
|---|---|---|---|---|
| 32 | S21 | 200 | 1 | 18.4 |
| 33 | S21 | 500 | 1 | 18.55 |

2.23g of K7598 was allowed to swell in 15.986g of deionized water for 30 minutes and the swollen gelatin was heated up to 36°C. The following ingredients were then added with stirring: 4.434g of a 20% aqueous solution of phthalazinone followed by 5 minutes stirring, then 22.20g of the silver behenate dispersion at a temperature of 36°C (for the surfactant used see table 16) followed by 10 minutes stirring, then 11.150g of an aqueous solution containing 5.55% of boric acid, 8.17% of R01 and 15.23% of ethanol was added and finally 1.0g of an aqueous solution containing 19.2% of formaldehyde and 6.75% of methanol.

The resulting silver behenate dispersions were then doctor blade-coated onto a 175µm thick subbed (subbing layer 1 described for COMPARATIVE EXAMPLE 5) polyethylene terephthalate support to produce the coating weights of silver given in table 17.

### Thermographic evaluation

The thermographic recording materials of REFERENCE EXAMPLES 27 and 28 and INVENTION EXAMPLES 1 and 2 were printed and the prints evaluated as described for REFERENCE EXAMPLES 1 to 10 and COMPARATIVE EXAMPLES 1 & 2. The maximum and minimum densities of the prints obtained with the thermographic recording materials of REFERENCE EXAMPLES 27 and 28 and INVENTION EXAMPLES 1 and 2 measured through a blue filter with a MACBETH™ TR924 densitometer for grey scale steps corresponding to data levels of 255 and 0 respectively are also given in table 117.

The light box tests were carried out on the thermographic recording materials of REFERENCE EXAMPLES 27 and 28 and INVENTION EXAMPLES 1 and 2 as described for REFERENCE EXAMPLES 1 to 10 and COMPARATIVE EXAMPLES 1 & 2. The results are summarized in table 17.

**Table 17:**

| Reference example number | AgB coverage [g/m²] | Surfactants | | fresh | | Light box: ΔDₘₐₓ/ΔDₘᵢₙ blue after 3d at 30°C/85% RH |
|---|---|---|---|---|---|---|
| | | Nr . | [Cl⁻] [ppm] | Dₘₐₓ blue | Dₘᵢₙ blue | |
| 27 | 3.74 | S01,S04,S16,S19 | 35-54 | 2.55 | 0.05 | +0.07/+0.02 |
| 28 | 3.66 | S01,S04,S16,S20 | 84 | 2.43 | 0.05 | +0.22/+0.02 |

| Invention example number | | | | | | |
|---|---|---|---|---|---|---|
| 1 | 3.66 | S01,S04,S16,S21 | 230 | 2.63 | 0.05 | -0.07/+0.01 |
| 2 | 3.40 | S01,S04,S16,S22 | 524 | 2.26 | 0.05 | +0.14/+0.01 |

The results of the thermographic evaluation of the thermographic recording material of REFERENCE EXAMPLES 27 and 28 and INVENTION EXAMPLES 1 and 2 show low increases in Dₘᵢₙ in archivability, indicating high stability, particularly in view of the subbing layer used which contains S16 with a very high concentration of chloride-ion. There is no significant diffference in light stability between the thermographic recording materials of REFERENCE EXAMPLES 27 and 28 and INVENTION EXAMPLES 1 and 2 indicating that up to a concentration of 524ppm the total chloride ion concentration in the surfactants present has no significant influence on the light stability of thermographic recording materials.

Having described in detail preferred embodiments of the current invention, it will now be apparent to those skilled in the art that numerous modifications can be made therein without departing from the scope of the invention as defined in the following claims.

## Claims

1. A process for producing a substantially light-insensitive thermographic recording material substantially exclusive of cationic surfactants in which at least one non-cationic surfactant is present, wherein said thermographic recording material comprises a support and a thermosensitive element containing a substantially light-insensitive silver salt of an aliphatic carboxylic acid known as a fatty acid, a reducing agent therefor in thermal working relationship therewith and a binder, comprising the steps of: producing an aqueous dispersion of said substantially light-insensitive silver salt of an aliphatic carboxylic acid known as a fatty acid; producing one or more aqueous coating compositions containing together said aqueous dispersion of the substantially light-insensitive silver salt of an aliphatic carboxylic acid known as a fatty acid, said reducing agent and said binder; and applying said one or more aqueous coating compositions to said support thereby forming after drying said thermosensitive element, **characterized in that** one or more of said aqueous dispersion of said substantially light-insensitive silver salt of an aliphatic carboxylic acid known as a fatty acid and said one or more aqueous coating compositions contain a non-cationic surfactant and all said non-cationic surfactants present in the thermographic recording material together have a non-fluoro-halide ion concentration of 1500 to 200ppm.

2. Production process according to claim 12, wherein said aqueous dispersion of said substantially light-insensitive organic silver salt is an aqueous dispersion of particles of substantially light-insensitive silver salt of an aliphatic carboxylic acid known as fatty acid including silver behenate in an aqueous medium produced by a process comprising the steps of: i) producing an aqueous dispersion of one or more organic acids including behenic acid and an anionic surfactant; ii) substantially neutralizing said organic acids with aqueous alkali thereby forming organic acid salts including a behenic acid salt; (iii) adding an aqueous solution of a silver salt to completely convert said organic acid salts into their silver salts including silver behenate, **characterized in that** said anionic surfactant is present in a molar ratio with respect to organic acid greater than 0.15 and said silver salt is added at a rate between 0.025mol/mol organic silver salt·min and 2.25mol/mol organic silver salt-min.

3. A substantially light-insensitive thermographic recording material obtained by the process of claim 1 or 2.

4. Substantially light-insensitive thermographic recording material according to claim 3, wherein all said non-cationic surfactants present together have a non-fluoro-halide ion concentration of 1000ppm or less.

5. Substantially light-insensitive thermographic recording material according to claim 3 or 4, wherein all said non-cationic surfactants present together have a metal ion concentration of 500 ppm or less.

6. Substantially light-insensitive thermographic recording material according to anyone of claims 3 to 5, wherein all said non-cationic surfactants present together have a metal ion concentration of 200ppm or less.

7. Substantially light-insensitive thermographic recording material according to any one of claims 3 to 6, wherein said non-fluoro halide ion is a chloride ion.

8. Substantially light-insensitive thermographic recording material according to any one of claims 3 to 7, wherein said binder is gelatin.

9. Substantially light-insensitive thermographic recording material according to any one of claims 3 to 8, wherein said thermosensitive element is provided with a protective layer.

10. Substantially light-insensitive thermographic recording material according to claim 9, wherein said protective layer contains a non-cationic surfactant.

11. Substantially light-insensitive thermographic recording material according to any one of claims 3 to 10, wherein a subbing layer is provided between said thermosensitive element and said support.

12. Substantially light-insensitive thermographic recording material according to claim 11, wherein said subbing layer contains a non-cationic surfactant.

13. Substantially light-insensitive thermographic recording material according to any one of claims 3 to 12, wherein said thermographic recording material is a black and white thermographic recording material.

14. Substantially light-insensitive thermographic recording material according to claim 3, wherein all said non-cationic surfactants present together have an alkali metal ion concentration of 200ppm or less.

## Patentansprüche

1. Ein Verfahren zur Herstellung eines wesentlich lichtunempfindlichen thermografischen Aufzeichnungsmaterials, das im Wesentlichen keine kationischen Tenside, wohl aber zumindest ein nicht-kationisches Tensid enthält, wobei das thermografische Aufzeichnungsmaterial einen Träger und ein wärmeempfindliches Element enthält, wobei das wärmeempfindliche Element ein wesentlich lichtunempfindliches Silbersalz einer als Fettsäure bekannten alifatischen Carbonsäure, ein Reduktionsmittel dafür in thermischer wirksamer Beziehung dazu und ein Bindemittel enthält, wobei das Verfahren durch folgende Schritte gekennzeichnet ist : Anfertigung einer wässrigen Dispersion des wesentlich lichtunempfindlichen Silbersalzes einer als Fettsäure bekannten alifatischen Carbonsäure, Herstellung einer oder mehrerer wässriger Gießzusammensetzungen, die zusammen die wässrige Dispersion des wesentlich lichtunempfindlichen Silbersalzes einer als Fettsäure bekannten alifatischen Carbonsäure, das Reduktionsmittel und das Bindemittel enthalten, und Auftrag der einen oder mehreren wässrigen Gießzusammensetzungen auf den Träger, wobei nach Trocknung das wärmeempfindliche Element erhalten wird, **dadurch gekennzeichnet, dass** die wässrige Dispersion des wesentlich lichtunempfindlichen Silbersalzes einer als Fettsäure bekannten alifatischen Carbonsäure und/oder die wässrige(n) Gießzusammensetzung(en) ein nicht-kationisches Tensid enthält (enthalten) und alle im thermografischen Aufzeichnungsmaterial enthaltenen nicht-kationischen Tenside ein Verhältnis von nicht-fluorhaltigen Halogenidionen von 1.500 bis 200 ppm aufweisen.

2. Herstellungsverfahren nach Anspruch 1, **dadurch gekennzeichnet, dass** die wässrige Dispersion des wesentlich lichtunempfindlichen organischen Silbersalzes eine wässrige Dispersion von Teilchen eines wesentlich lichtunempfindlichen Silbersalzes einer als Fettsäure bekannten alifatischen Carbonsäure, wozu Silberbehenat zählt, in einem wässrigen Medium ist, die durch ein durch die nachstehenden Schritte gekennzeichnetes Verfahren angefertigt wird : (i) Anfertigung einer wässrigen Dispersion, die eine oder mehrere organische Säuren, wozu Behensäure zählt, und ein anionisches Tensid enthält, (ii) wesentliches Neutralisieren der organischen Säuren mit wässrigem Alkali, wobei Salze einer organischen Säure, wozu das Salz von Behensäure zählt, gebildet werden, und (iii) Zugabe einer wässrigen Lösung eines Silbersalzes, um die Salze der organischen Säure völlig in ihre Silbersalze, wozu Silberbehenat zählt, umzuwandeln, **dadurch gekennzeichnet, dass** das anionische Tensid in einem Molverhältnis, bezogen auf die organische Säure, von mehr als 0,15 verwendet und das Silbersalz bei einer Geschwindigkeit zwischen 0,025 Mol pro Mol organisches Silbersalz pro Minute und 2,25 Mol pro Mol organisches Silbersalz pro Minute zugesetzt wird.

3. Ein nach dem in Anspruch 1 oder 2 definierten Verfahren hergestelltes wesentlich lichtunempfindliches thermografisches Aufzeichnungsmaterial.

4. Wesentlich lichtunempfindliches thermografisches Aufzeichnungsmaterial nach Anspruch 3, **dadurch gekennzeichnet, dass** alle nicht-kationischen Tenside zusammen ein Verhältnis von nicht-fluorhaltigen Halogenidionen von höchstens 1.000 ppm aufweisen.

5. Wesentlich lichtunempfindliches thermografisches Aufzeichnungsmaterial nach Anspruch 3 oder 4, **dadurch gekennzeichnet, dass** alle nicht-kationischen Tenside zusammen ein Metallionenverhältnis von höchstens 500 ppm aufweisen.

6. Wesentlich lichtunempfindliches thermografisches Aufzeichnungsmaterial nach einem der Ansprüche 3 bis 5, **dadurch gekennzeichnet, dass** alle nicht-kationischen Tenside zusammen ein Metallionenverhältnis von höchstens 200 ppm aufweisen.

7. Wesentlich lichtunempfindliches thermografisches Aufzeichnungsmaterial nach einem der Ansprüche 3 bis 6, **dadurch gekennzeichnet, dass** das nicht-fluorhaltige Halogenidion ein Chloridion ist.

8. Wesentlich lichtunempfindliches thermografisches Aufzeichnungsmaterial nach einem der Ansprüche 3 bis 7, **dadurch gekennzeichnet, dass** das Bindemittel Gelatine ist.

9. Wesentlich lichtunempfindliches thermografisches Aufzeichnungsmaterial nach einem der Ansprüche 3 bis 8, **dadurch gekennzeichnet, dass** das wärmeempfindliche Element mit einer Schutzschicht versehen ist.

10. Wesentlich lichtunempfindliches thermografisches Aufzeichnungsmaterial nach Anspruch 9, **dadurch gekennzeichnet, dass** die Schutzschicht ein nicht-kationisches Tensid enthält.

11. Wesentlich lichtunempfindliches thermografisches Aufzeichnungsmaterial nach einem der Ansprüche 3 bis 10, **dadurch gekennzeichnet, dass** zwischen das wärmeempfindliche Element und den Träger eine Haftschicht eingefugt ist.

12. Wesentlich lichtunempfindliches thermografisches Aufzeichnungsmaterial nach Anspruch 11, **dadurch gekennzeichnet, dass** die Haftschicht ein nicht-kationisches Tensid enthält.

13. Wesentlich lichtunempfindliches thermografisches Aufzeichnungsmaterial nach einem der Ansprüche 3 bis 12, **dadurch gekennzeichnet, dass** das thermografische Aufzeichnungsmaterial ein thermografisches Schwarzweiß-Aufzeichnungsmaterial ist.

14. Wesentlich lichtunempfindliches thermografisches Aufzeichnungsmaterial nach Anspruch 3, **dadurch gekennzeichnet, dass** alle nicht-kationischen Tenside ein Alkalimetallionenverhältnis von höchstens 200 ppm aufweisen.

## Revendications

1. Procédé pour la production d'un matériau d'enregistrement thermographique essentiellement non photosensible dans lequel on exclut essentiellement des agents tensioactifs cationiques et dans lequel est présent au moins un agent tensioactif non cationique, ledit matériau d'enregistrement thermographique comprenant un support et un élément thermosensible contenant un sel d'argent essentiellement non photosensible d'un acide carboxylique aliphatique désigné par l'expression « acide gras », un agent de réduction pour ledit sel en relation de travail thermique avec lui et un liant, comprenant les étapes consistant à : procurer une dispersion aqueuse dudit sel d'argent essentiellement non photosensible d'un acide carboxylique aliphatique désigné par l'expression « acide gras » ; produire une ou plusieurs compositions d'enduction aqueuses contenant, de manière conjointe, ladite dispersion aqueuse du sel d'argent essentiellement non photosensible d'un acide carboxylique aliphatique désigné par l'expression « acide gras », ledit agent de réduction et ledit liant ; et appliquer ladite ou lesdites compositions d'enduction aqueuse sur ledit support pour ainsi obtenir, après le séchage, ledit élément thermosensible, **caractérisé en ce qu'**une ou plusieurs desdites dispersions aqueuses dudit sel d'argent essentiellement non photosensible d'un acide carboxylique aliphatique désigné par l'expression acide gras et lesdites une ou plusieurs compositions d'enduction aqueuse contenant un agent tensioactif non cationique et la totalité desdits agents tensioactifs non cationiques présents dans le matériau d'enregistrement thermographique possèdent ensemble une concentration en ions halogénures de type non fluoro de 1500 à 200 ppm.

2. Procédé de protection selon la revendication 1, dans lequel ladite dispersion aqueuse dudit sel d'argent organique essentiellement non photosensible est une dispersion aqueuse de particules d'un sel d'argent essentiellement non photosensible d'un acide carboxylique aliphatique désigné par l'expression « acide gras », y compris le béhénate d'argent, dans un milieu aqueux, que l'on obtient via un procédé comprenant les étapes consistant à : i) préparer une dispersion aqueuse d'un ou de plusieurs acides organiques, y compris l'acide béhénique, et d'un agent tensioactif anionique ; ii) soumettre lesdits acides organiques à une neutralisation substantielle avec des alcalis aqueux pour ainsi obtenir des sels d'acides organiques, y compris un sel d'acide béhénique ; iii) ajouter une solution aqueuse d'un sel d'argent pour transformer complètement lesdits sels d'acides organiques en leurs sels d'argent, y compris le béhénate d'argent, **caractérisé en ce que** ledit agent tensioactif anionique est présent dans un rapport molaire par rapport à l'acide organique supérieur à 0,15, et ledit sel d'argent est ajouté à un débit entre 0,025 mole/mole de sel d'argent organique par minute et 2,25 moles/mole de sel d'argent organique par minute.

3. Matériau d'enregistrement thermographique essentiellement non photosensible que l'on obtient via le procédé selon la revendication 1 ou 2.

4. Matériau d'enregistrement thermographique essentiellement non photosensible selon la revendication 3, dans lequel tous lesdits agents tensioactifs non cationiques présents possèdent ensemble une concentration en ions halogénures de type non fluoro de 1000 ppm ou moins.

5. Matériau d'enregistrement thermographique essentiellement non photosensible selon la revendication 3 ou 4, dans lequel tous lesdits agents tensioactifs non cationiques présents possèdent ensemble une concentration en ions métalliques de 500 ppm ou moins.

6. Matériau d'enregistrement thermographique essentiellement non photosensible selon l'une quelconque des revendications 3 à 5, dans lequel tous lesdits agents tensioactifs non cationiques présents possèdent ensemble une concentration en ions métalliques de 200 ppm ou moins.

7. Matériau d'enregistrement thermographique essentiellement non photosensible selon l'une quelconque des revendications 3 à 6, dans lequel ledit ion halogénure de type non fluoro est un ion chlorure.

8. Matériau d'enregistrement thermographique essentiellement non photosensible selon l'une quelconque des revendications 3 à 7, dans lequel ledit liant est de la gélatine.

9. Matériau d'enregistrement thermographique essentiellement non photosensible selon l'une quelconque des revendications 3 à 8, dans lequel ledit élément thermosensible est muni d'une couche de protection.

10. Matériau d'enregistrement thermographique essentiellement non photosensible selon la revendication 7, dans lequel ladite couche de protection contient un agent tensioactif non cationique.

11. Matériau d'enregistrement thermographique essentiellement non photosensible selon l'une quelconque des revendications 3 à 10, dans lequel on prévoit une couche adhérente entre ledit élément thermosensible et ledit support.

12. Matériau d'enregistrement thermographique essentiellement non photosensible selon la revendication 11, dans lequel ladite couche adhérente contient un agent tensioactif non cationique.

13. Matériau d'enregistrement thermographique essentiellement non photosensible selon l'une quelconque des revendications 3 à 12, dans lequel ledit matériau d'enregistrement thermographique est un matériau d'enregistrement thermographique en noir et blanc.

14. Matériau d'enregistrement thermographique essentiellement non photosensible selon la revendication 3, dans lequel tous lesdits agents tensioactifs non cationiques présents possèdent ensemble une concentration en ions de métaux alcalins de 200 ppm ou moins.
